



US006110758A

**United States Patent** [19]

Estrera et al.

[11] **Patent Number:** **6,110,758**[45] **Date of Patent:** **Aug. 29, 2000**

[54] **TRANSMISSION MODE PHOTOCATHODE WITH MULTILAYER ACTIVE LAYER FOR NIGHT VISION AND METHOD**

[75] Inventors: **Joseph P. Estrera**, Dallas; **Keith T. Passmore**, Rowlett; **Timothy W. Sinor**, Plano, all of Tex.

[73] Assignee: **Litton Systems, Inc.**, Beverly Hills, Calif.

[21] Appl. No.: **09/435,880**

[22] Filed: **Nov. 8, 1999**

**Related U.S. Application Data**

[62] Division of application No. 08/527,688, Sep. 13, 1995.

[51] **Int. Cl. 7** ..... **H01L 21/00**

[52] **U.S. Cl.** ..... **438/93; 438/20; 438/64; 438/125; 438/118**

[58] **Field of Search** ..... **438/20, 64, 93, 438/125, 118**

[56] **References Cited****U.S. PATENT DOCUMENTS**

|           |         |                      |           |
|-----------|---------|----------------------|-----------|
| 3,696,262 | 10/1972 | Antypas              | 313/94    |
| 3,814,996 | 6/1974  | Enstrom              | 357/30    |
| 3,868,523 | 2/1975  | Klopfur et al.       | 313/94    |
| 3,894,258 | 7/1975  | Butterwick           | 313/102   |
| 3,906,277 | 9/1975  | Schade               | 313/365   |
| 3,914,136 | 10/1975 | Kressel              | 148/171   |
| 3,951,698 | 4/1976  | Wilson et al.        | 148/33.4  |
| 3,960,620 | 6/1976  | Ettenberg            | 148/175   |
| 4,096,511 | 6/1978  | Gurnell et al.       | 357/30    |
| 4,115,223 | 9/1978  | Thrush               | 204/129.6 |
| 4,563,614 | 1/1986  | Howorth              | 313/524   |
| 4,616,248 | 10/1986 | Khan et al.          | 357/30    |
| 4,644,221 | 2/1987  | Gutierrez et al.     | 313/373   |
| 4,829,355 | 5/1989  | Munier et al.        | 357/30    |
| 4,980,312 | 12/1990 | Harris et al.        | 437/90    |
| 5,146,296 | 9/1992  | Huth                 | 357/19    |
| 5,268,570 | 12/1993 | Kim                  | 250/214   |
| 5,378,640 | 1/1995  | Kim                  | 437/5     |
| 5,404,026 | 4/1995  | Mariella, Jr. et al. | 257/10    |
| 5,506,402 | 4/1996  | Estrera              | 250/414   |

5,747,862 5/1998 Kishino et al. ..... 257/436

**OTHER PUBLICATIONS**

Stringfellow, G. B., "Lattice Parameters and Crystal Structure of Indium-Gallium-Arsenide," *Properties of Lattice-Matched and Strained Indium-Gallium-Arsenide*, P. Bhattacharya, Edit, Institution of Electrical Engineers, London, United Kingdom, 1993.

Takahashi, N.S., "Lattice Parameters, Molecular and Crystal Densities of Aluminun-Gallium-Arsenide," *Properties of Aluminum-Gallium-Arsenide*, S. Adachi, Editor, Institution of Electrical Engineers, London, United Kingdom, 1993.

D.G. Fisher, R.E. Enstrom, J.S. Escher, H.F. Gossenberger, and J.R. Appert, Photoemission Characteristics of Transmission-Mode Negative Electron Affinity GaAs and (In,Ga)As Vapor-Grown Structures, *IEEE Transactions on Electron Devices*, vol. ED-21, No. 10 pp. 641-649 (1974).

R.E. Nahory, M.A. Pollack, and J.C. DeWinter, Growth and characterization of liquid-phase epitaxial  $In_xGa_{1-x}As$ , *Journal of Applied Physics*, vol. 46, No. 2 pp. 775-782 (1975).

A.H. Sommer, The element of luck in research-photocathodes 1930 to 1980, *J. Vac. Sci. Technol. A* 1(2), pp. 119-124, Apr.-Jun. 1983.

G. Vergara, L.J. Gomez, J. Capmany and M.T. Montojo, Adsorption kinetics of cesium and oxygen on GaAs(100), *Surface Science* 278 pp. 131-145 (1992).

(List continued on next page.)

*Primary Examiner*—David Nelms

*Assistant Examiner*—Quoc Hoang

*Attorney, Agent, or Firm*—Baker Botts LLP

[57]

**ABSTRACT**

An improved photocathode and image intensifier tube are disclosed along with a method for making both the tube and photocathode. The disclosed photocathode and image intensifier tube have an active layer comprising two or more sublayers. The first sublayer has a first concentration of a group III-V semiconductor compound while the second sublayer has a second concentration of the group III-V semiconductor compound. The multilayer active layer is coupled to a window layer.

**20 Claims, 2 Drawing Sheets**



## OTHER PUBLICATIONS

- D.G. Fisher, R.E. Enstrom, J.S. Escher, and B.F. Williams, Photoelectron surface escape probability of (Ga,In)As: Cs-O In the 0.9 to  $\approx 1.6 \mu\text{m}$  range\*, *J. Appl. Phys.* vol. 43, No. 9, pp. 3815–3823 (1972).
- R.L. Bell, L.W. James, and R.L. Moon, Transferred electron photoemission from InP†, *Appl. Phys. Letters*, vol. 25, No. 11, pp. 645–646 (1974).
- J.S. Escher and R. Sankaran, Transferred Electron Photoemission to  $1.4 \mu\text{m}$ , *Appl. Phys. Lett.* 29, 87 (1976).
- J.S. Escher, P.E. Gregory, S.B. Hyder, and R. Sankaran, Transferred-electron photoemission to  $1.65 \mu\text{m}$  from InGaAs<sup>o</sup>, *J. Appl. Phys.* 49(4), pp. 2591–2592 (1978).
- P.E. Gregory, J.S. Escher, S.B. Hyder, Y.M. Hwang, and G.A. Antypas, Field-assisted minority carrier electron transport across a p-InGaAs/ p-InP heterojunction<sup>o</sup>, *J. Vac. Sci. Technol.* 15(4), pp. 1483–1487 (1978).
- J.S. Escher, R.L. Bell, P.E. Gregory, S.Y. Hyder, T.J. Maloney, and G.A. Antypas, Field-Assisted Semiconductor Photoemitters for the 1–2  $\mu\text{m}$  Range, *IEEE Transactions on Electron Devices* ED-27, No. 7, pp. 1244–1250 (1980).
- J.S. Escher, P.E. Gregory, S.B. Hyder, R.R. Saxena, and R.L. Bell, Photoelectric Imaging in the 0.9–1.6 Micron Range\*, *IEEE Electron Device Letters*, vol. EDL-2, No. 5, pp. 123–125 (1981).
- K. Costello, G. Davis, R. Weiss, and V. Aebi, SPIE Proceedings; Electron Image Tubes and Image Intensifiers II, vol. 1449 (1991).
- I.P. Csorba, Recent advancements in the field of image intensification: the generation 3 wafer tube, *Applied Optics*, vol. 18(14), pp. 2440–2444 (Jul. 1979).
- I.P. Csorba, Current Status of Image Intensification, *Milttronics*, pp. 2–11 (Mar./May 1981).
- I.P. Csorba, Current Status and Performance Characteristics of Night Vision Aids, *Opto-Electronic Imaging*, Chapter 3, pp. 34–63 (1985).
- K.A. Costello, V.W. Aebi and H.F. MacMillan, Imaging GaAs Vacuum Photodiode with 40% Quantum Efficiency at 530 nm, *SPIE vol. 1243 Electron Image Tubes and Image Intensifiers* pp. 99–104 (1990).
- A.A. Narayanan, D.G. Fisher, L.P. Erickson and G.D. O'Clock, Negative electron affinity gallium arsenide photocathode grown by molecular beam epitaxy, *J. Appl. Phys.* vol. 56(6) pp. 1886–1887 15 Sep. 1984.



FIG. 1



FIG. 2



FIG. 3



## TRANSMISSION MODE PHOTOCATHODE WITH MULTILAYER ACTIVE LAYER FOR NIGHT VISION AND METHOD

### CROSS REFERENCE TO RELATED APPLICATIONS

This application is a divisional of U.S. application Ser. No. 08/527,688, filed Sep. 13, 1995, by Joseph P. Estrera, Keith T. Passmore and Timothy W. Sinor and entitled "TRANSMISSION MODE PHOTOCATHODE WITH MULTILAYER ACTIVE LAYER FOR NIGHT VISION AND METHOD."

### TECHNICAL FIELD OF THE INVENTION

This invention relates generally to night vision systems, and more particularly, to an improved photocathode and image intensifier tube and a method for making the same.

### BACKGROUND OF THE INVENTION

Detection and imaging out to the near infrared (wavelengths greater than 940 nm) have been a weak point of standard image intensifier and night vision systems. Standard night vision systems using Gen II (S-20, S-25) and Gen III (GaAs NEA) based photocathodes have little or no photosensitivity beyond wavelengths of 940 nm. However, sensitivity beyond those wavelengths is desirable. Night sky radiation begins to increase dramatically beyond 950 nm wavelength and most existing detectors and imagers cannot observe this increased night sky irradiance. More importantly, most standard photocathode systems cannot detect or utilize the active imaging capability of near infrared based lasers such as the Nd:YAG laser with 1.064  $\mu\text{m}$  monochromatic radiation.

Recently, non-field assisted transmission mode photocathodes capable of imaging Nd:YAG laser radiation have been developed by Varo, Inc. These devices take advantage of an active layer of indium-gallium-arsenide coupled with an aluminum-gallium-arsenide window layer. Although these devices have sensitivity to near infrared wavelengths, increased sensitivity would be desirable for some applications.

Moreover, it would be desirable to have a photocathode with photosensitivity in the near infrared range of 1 to 1.7  $\mu\text{m}$ . In particular, certain designators and laser rangefinders used in military applications employ erbium-doped glass lasers which produce radiation with a wavelength of between 1.4 and 1.5  $\mu\text{m}$ . Existing image intensifiers and night vision systems are not capable of detecting radiation with wavelengths in this range.

In photocathodes with an indium-gallium-arsenide active layer, detecting longer wavelengths requires the indium-gallium-arsenide active layer to have a high percentage of indium. For example, it is believed that a photocathode capable of detecting radiation from an erbium-doped glass laser would require an indium percentage in the active layer between forty and sixty percent. As the percentage of indium increases, however, crystal stress increases due to variations between the lattice constant of the active layer and the lattice constant of the window layer.

When the indium concentration reaches such a high level, degradation in crystal quality is significant. Increased crystal stress due to the mismatch of the lattice constants between the window and active layers causes both light scatter and electron scatter. Irregularities in the lattice due to crystal stress cause light scatter. In an irregular lattice, photons are

not absorbed properly, but instead are reflected and scattered within the crystal. Lattice irregularities also prevent electrons from easily escaping the lattice and instead tend to cause electrons to scatter. These effects combine to sufficiently lower the quantum efficiency of such a device so as to make it unacceptable for a standard image intensifier in a night vision system.

### SUMMARY OF THE INVENTION

The present invention avoids the limitations of existing photocathodes and image intensifier tubes by using an improved photocathode having an active layer with multiple sublayers. An improved image intensifier tube and photocathode are disclosed along with a method for making both. One aspect of the invention is an improved photocathode having a window layer adjacent to an active layer. The active layer comprises two or more sublayers where at least one sublayer has a first concentration of a group III-V semiconductor compound and another sublayer has a second concentration of the group III-V semiconductor compound.

The invention has many important technical advantages. One advantage is that the photocathode has a higher quantum efficiency than many existing photocathodes. By controlling the concentration of a particular group III-V semiconductor compound in each sublayer such that the energy band of each sublayer decreases as the sublayers get farther away from the window layer, a cascade effect is created. By placing the sublayer with the highest energy adjacent to the window layer and then decreasing the energy of each succeeding sublayer, it is believed that a cascade effect is created such that the movement of electrons from high energy bands to low energy bands causes additional electrons to be generated in succeeding sublayers, thus increasing the total number of electrons generated by the active layer in response to radiation. This effect also allows the photocathode to be sensitive to both visible and near infrared radiation without the complications of high energy electrons trying to travel through bulk low energy based material which has short diffusion lengths.

The multilayer structure of the active layer substantially reduces crystal stress and allows at least a portion of the active layer to have a higher percentage group III-V semiconductor compound which would be unattainable in a single layer device. For example, by gradually increasing the percentage of indium in sublayers moving away from the window layer, a higher indium concentration can be achieved without causing crystal stress. The higher indium concentration in outer sublayers allows the invention to achieve higher sensitivity to near-infrared radiation in a device with good quantum efficiency.

For example, the invention can be used to achieve sensitivity in a photocathode and image intensifier to near infrared radiation in the 1.4-1.5  $\mu\text{m}$  range. Such sensitivity is advantageous for use of night vision equipment with military designators and laser rangefinders employing erbium-doped glass lasers. By carefully varying the concentration of a group III-V semiconductor compound in various sublayers, and/or varying the thickness of various sublayers, one can tune a photocathode to have narrow band spectral sensitivity. These advantages are all achieved without sacrificing compatibility with existing Gen III image intensifier format. Gen III manufacturing processes can be used to produce the photocathode and image intensifiers. The resulting photocathode is also advantageous in that it is a transmission mode device that is non-field assisted.

Applications of the invention include night vision systems, military systems, CCD camera technology, gated

imaging technology, and scientific applications involving the detection of near-infrared radiation.

#### BRIEF DESCRIPTION OF THE DRAWINGS

For a more complete understanding of the present invention, and the advantages thereof, reference is now made to the following descriptions taken in conjunction with the accompanying drawings, in which:

FIG. 1 illustrates a photocathode made in accordance with the invention;

FIG. 2 illustrates a wafer structure used to produce the photocathode of FIG. 1;

FIG. 3 illustrates an image intensifier tube made in accordance with the invention; and

FIG. 4 is a graph comparing the spectral response of conventional Gen II and Gen III image intensifier tubes with an example image intensifier tube constructed in accordance with the teachings of the present invention.

#### DETAILED DESCRIPTION OF THE INVENTION

The preferred embodiment of the present invention and its advantages are best understood by referring to FIGS. 1 through 4 of the drawings, like numerals being used for like and corresponding parts of the various drawings.

FIG. 1 illustrates a cross-sectional side view of one example of a photocathode 10 constructed in accordance with the teachings of the present invention. Photocathode 10 comprises face plate 12, anti-reflection coating 14, window layer 16, active layer 18, and electrode 26. Active layer 18 further comprises first sublayer 20, second sublayer 22 and third sublayer 24.

Face plate 12 is made of glass and is bonded to anti-reflection coating 14. Anti-reflection coating 14 comprises a first layer of silicon nitride which serves as an anti-reflection coating and a second layer of silicon dioxide which provides thermal protection and a bonding layer for coupling window layer 16 to face plate 12 during the thermal bonding process described below in connection with FIG. 2. The thickness of the silicon nitride and silicon dioxide layers is approximately 1000 angstroms each.

Anti-reflection coating 14 connects to window layer 16. Window layer 16 preferably comprises one or more group III-V semiconductor compounds. In this example, window layer 16 comprises aluminum-gallium-arsenide (AlGaAs). Window layer 16 serves as a short-wavelength cutoff filter for incoming light into photocathode 10, a barrier and reflector for electrons trying to go in the direction of the interface between window layer 16 and active layer 18, and a supporting and thermal protective layer for active layer 18. Window layer 16 has a thickness of approximately 0.8–1.0  $\mu\text{m}$  and has a p-type doping level of  $1\text{--}3 \times 10^{18} \text{ cm}^{-3}$ . The aluminum composition and thickness of window layer 16 may be adjusted to obtain the desired amount of short wavelength radiation through that layer.

Active layer 18 comprises three sublayers which are each 0.5–1.0  $\mu\text{m}$  thick. Active layer 18 comprises one or more group III-V semiconductor compounds. In this example, active layer 18 comprises indium gallium arsenide (InGaAs). The indium concentration of each sublayer increases beginning at first sublayer 20 and ending at third sublayer 24. Given a formula of  $\text{In}_x\text{Ga}_{1-x}\text{As}$ , the percent concentration of indium in a given layer is governed by the formula  $100 \times x$ . In this example, first sublayer 20 has a five percent indium concentration, second sublayer 22 has a ten

percent indium concentration and third sublayer 24 has a fifteen percent indium concentration. Thus, the indium concentration is graded such that the concentration increases as the sublayers get farther away from window layer 16.

Electrode 26 is coupled to face plate 12, anti-reflection coating 14, window layer 16 and active layer 18. Electrode 26 is a chrome gold electrode.

In operation, photons enter photocathode 10 through face plate 12 and pass through anti-reflection coating 14 and window layer 16. As the photons strike active layer 18, electrons are generated and emitted from the surface of active layer 18.

The sublayer structure of active layer 18 can be arranged in a way so as to filter various wavelengths. Layers with low indium concentrations such as sublayer 20 absorb photons with short wavelengths and generate electrons in response to such absorption. Photons with longer wavelengths pass through sublayers such as first sublayer 20 with low indium concentration. At second sublayer 22, photons with slightly longer wavelengths are absorbed and generate electrons, while even longer wavelengths pass through to third sublayer 24. Third sublayer 24 generates electrons in response to photons having even longer wavelengths.

The compositional grading of active layer 18 reduces crystal stress between window layer 16 and active layer 18. Reducing crystal stress allows near infrared sensitivity to be increased with high quantum efficiency. The reduction in crystal stress allows more photogenerated electrons to travel through an undamaged crystal lattice of the photocathode. These benefits can be achieved because the sublayers nearest to window layer 16 have a lower indium concentration and therefore have a lattice constant closer to that of window layer 16. By gradually increasing indium concentration, lattice mismatch effects between window layer 16 and active layer 18 are drastically reduced. By raising the concentration of indium in the outer sublayers, better sensitivity to near-infrared radiation can be achieved.

Compositional grading also allows formation of an electronic band structure in photocathode 10 which causes photogenerated electrons to cascade from high to low energy conduction subbands. Sublayers with lower indium concentration have higher energy. In this example, first sublayer 20 has higher energy than second sublayer 22 and second sublayer 22 has higher energy than third sublayer 24. This compositional grading causes photogenerated electrons to cascade down their respective higher energy conduction subbands to lower energy conduction subbands in sublayers with higher indium concentration. The overall effect of the multilayer construction of active layer 18 is to easily transport electrons generated by high energy radiation (visible light) to lower energy based material (high indium concentration layers) for escape to the surface of photocathode 10. Compositional grading thus allows photocathode 10 to have the ability to be sensitive to both visible and near infrared radiation without the complication of high energy electrons trying to travel through bulk low energy (high indium concentration) InGaAs which has short diffusion lengths (less than 1.0  $\mu\text{m}$ ).

Selectively arranging the thicknesses of the sublayers of active layer 18 along with selective doping allows photocathode 10 to be made to have narrow band spectral sensitivities. This feature is attractive for laser imaging applications.

The method of making photocathode 10 can best be understood by referring to FIG. 2 in conjunction with FIG. 1. FIG. 2 illustrates a cross-sectional side view of a multi-

layer wafer **28** used in making photocathode **10**. Wafer **28** comprises substrate **30**, stop layer **32**, active layer **18**, window layer **16**, and cap layer **34**. Active layer **18** further comprises first sublayer **20**, second sublayer **22**, and third sublayer **24**. Photocathode **10** is preferably fabricated using steps similar to those used in standard Gen III processes.

Wafer **28** is an epitaxially grown wafer structure. It may be formed, for example, using processes such as metal organic chemical vapor deposition (MOCVD), molecular beam epitaxy (MBE) or metal organic molecular beam epitaxy (MOMBE). The fabrication process for the illustrated embodiment begins by using a commercially available single crystal gallium arsenide substrate **30** with a low defect density. Substrate **30** will be the foundation and support for the epitaxial growth of subsequent layers. Another type of substrate **30** could also be used.

Stop layer **32** is grown on substrate **30**. Stop layer **32** is made of AlGaAs. In later processing steps, substrate **30** will be etched off; stop layer **32** prevents further etching into subsequent layers at that time. Stop layer **32** may have, for example, a thickness between approximately 1.0 and 1.5  $\mu\text{m}$  and an aluminum composition of forty-five percent or greater. The aluminum composition is chosen to ensure that the selective etch used to remove substrate **32** will terminate at stop layer **32**. Other materials could be used to form stop layer **32**.

Active layer **18** is then epitaxially grown on top of stop layer **32**. Active layer **18** in this example has a thickness of between 1.5 and 3.0  $\mu\text{m}$ . As described above, active layer **18** comprises two or more sublayers. In this example, active layer **18** comprises first sublayer **20**, second sublayer **22**, and third sublayer **24**, which are each 0.5 to 1.0  $\mu\text{m}$  thick. Here, active layer **18** is InGaAs. Third sublayer **24** is first grown followed by second sublayer **22** and first sublayer **20**. Each sublayer of active layer **18** is doped using a p-type impurity (such as Zn) at levels of between 1 and  $9 \times 10^{18} \text{ cm}^{-3}$  to provide electron transportability through active layer **18** and reduction of the surface work function of active layer **18** for surface electron escapability. In this example, the doping of the sublayers ranges from low doping ( $2 \times 10^{18} \text{ cm}^{-3}$ ) for first sublayer **20** to higher doping ( $6 \times 10^{18} \text{ cm}^{-3}$ ) for a third sublayer **24**. This doping construction allows for increased electron transport due to longer diffusion lengths. The indium concentration of each sublayer varies as discussed above.

Window layer **16** is then epitaxially grown on active layer **18**. Window layer **16** in this embodiment is AlGaAs and is doped as described above.

Finally, cap layer **34** is epitaxially grown on top of window layer **16**. Cap layer **34**, for example, may be formed of gallium arsenide. Cap layer **34** serves to protect window layer **16** during the cool down of the full epitaxial structure and/or during wafer transport.

After wafer **28** is grown, cap layer **34** is removed with a proper selective etch to expose window layer **16**. Coating layer **14**, as illustrated in FIG. 1, is then applied to the exposed surface of window layer **16**. Coating layer **14** itself comprises an anti-reflection layer and a thermal bonding layer as described above. After coating layer **14** has been applied to the surface of window layer **16**, the full wafer structure is heated during a thermal compression bonding of the wafer structure to face plate **12**.

After face plate **12** has been bonded to the wafer structure, substrate **30** and stop layer **32** are selectively etched to expose active layer **18**. Using standard thin film techniques, electrode **26** is formed and coupled to face plate **12**, active

layer **18**, window layer **16**, and coating layer **14**. In this embodiment, electrode **26** is applied to the circumference of each layer as illustrated in FIG. 1.

Photocathode **10** is then etched to remove residual gas, moisture, and oxides that have attached to the surface of active layer **18** during previous processing. Photocathode **10** is next placed into a vacuum system and heated to clean the surface of active layer **18**. To activate active layer **18**, cesium and oxygen vapor are evaporated onto its surface. During evaporation, input light enters the surface of active layer **18** producing an output current measured from electrode **26**. Cesium and oxygen vapors are further applied until achieving a maximum electrode current. At this point, the evaporation process stops and photocathode **10** may then be sealed into an image intensifier tube such as that described below in connection with FIG. 3.

It should be understood that the invention is not limited to the illustrated structures and that a number of substitutions can be made without departing from the scope and teachings of the present invention. For example, electrode **26** is a chrome gold electrode. Chrome-gold was chosen for this embodiment because it aids in vacuum sealing of image intensifier tubes such as those discussed in connection with FIG. 3. Electrode **26** could be made of a different material.

Face plate **12** is formed from Corning 7056 glass. 7056 glass or its equivalent is advantageously used because its thermal expansion coefficient matches closely with the thermal expansion coefficient of the remainder of photocathode **10**. Face plate **12** could be made of another material such as quartz or a fiberoptic material.

Anti-reflection coating **14** could be omitted in some applications. In addition, the various sublayers of anti-reflection coating **14** could be made of different materials and/or have different thicknesses.

Depending upon the material used for active layer **18**, window layer **16** could be made of a different semiconductor material. A semiconductor material should preferably be chosen having a lattice constant close to that of first sublayer **20** of active layer **18**. Here, window layer **16** is comprised of two group III-V semiconductor compounds—AlAs and GaAs. Other group III-V semiconductor compounds could be used and more than two such compounds could be used. Window layer **16** could also have a different thickness and/or a different doping.

The disclosed embodiment has three sublayers in active layer **18**. Active layer **18** could have only two sublayers or more than three sublayers. Each of the sublayers of active layer **18** could be doped differently or have different thicknesses. Different group III-V semiconductor materials could also be used for active layer **18**. Here, the group III-V semiconductor compounds InAs and GaAs have been used. Other group III-V semiconductor compounds could be used and more than two group III-V semiconductor compounds could be used to form active layer **18**.

In this example, the sublayers of active layer **18** have an InAs concentration of five percent, ten percent, and fifteen percent. These percentages can be varied. For example, to produce a photocathode capable of detecting radiation produced by an erbium-doped glass laser (1.4–1.5  $\mu\text{m}$ ), one of the InGaAs sublayers should have an indium concentration of between fifty and sixty percent. The number of sublayers and concentration for each sublayer will vary depending upon the desired application.

Photocathode **10** may advantageously be used for image intensifier tubes commonly used for night vision systems. FIG. 3 illustrates an image intensifier tube **36** made in

accordance with the invention. Image intensifier tube 36 comprises photocathode 10 which is operable to emit electrons in response to photons emitted from an image. A display apparatus couples to photocathode 10 and is operable to transform the emitted electrons into a visible light image. In the embodiment illustrated in FIG. 3, the display apparatus comprises a multichannel plate 38 adjacent to photocathode 10, a phosphor screen 40 adjacent to multichannel plate 38 and a fiberoptic anode 42 adjacent to phosphor screen 40.

Multichannel plate 38 may comprise, for example, a thin wafer having several parallel hollow glass fibers, each oriented slightly off axis with respect to incoming electrons. In the embodiment of FIG. 3, multichannel plate 38 multiplies incoming electrons with a cascade of secondary electrons through the channels by applying a voltage across the two faces 44, 46 of multichannel plate 38. The surface of phosphor screen 40 receives electrons from multichannel plate 38 and phosphor screen 40 generates a visible light image. Fiberoptic anode 42 translates the image produced by phosphor screen 40 using, for example, fiberoptic bundles to form a translated image that is visible to an observer.

FIG. 3 further illustrates the operation of image intensifier tube 36. An image 48 emits photons 50 which are directed onto a surface of photocathode 10. Photocathode 10 transforms photons 50 into electrons 52 which gain energy from an electric field between photocathode 10 and multichannel plate 38. Multichannel plate 38 multiplies the incoming electrons 52 with a cascade of secondary electrons to form multiplied electrons 54 which are then transported by a high energy electric field between multichannel plate 38 and the surface of phosphor screen 40. As electrons strike phosphor screen 40, they generate a visible light image which is then translated by fiberoptic anode into an output image 56 visible to an observer.

FIG. 4 illustrates a graph comparing the spectral response of standard Gen II and Gen III image intensifier tubes with an image intensifier tube 36 constructed in accordance with the teachings of the present invention. The embodiment of photocathode 10 illustrated in FIG. 1 was used for the image intensifier tube 36. This embodiment has high sensitivity at the 1.06  $\mu\text{m}$  wavelength. This embodiment is thus useful for applications where imaging of an Nd:YAG laser is desired. This graph provides only one example of the spectral responses that can be achieved when using image intensifier tubes constructed using the techniques of the invention.

Although the present invention and its advantages have been described in detail, it should be understood that various changes, substitutions and alterations can be made therein without departing from the spirit and scope of the invention as defined by the appended claims.

What is claimed is:

1. A method of making a photocathode, comprising:

forming a wafer structure according to the steps of:

growing a first sublayer having a first concentration of a group III-V semiconductor compound, and  
growing a second sublayer having a second concentration of the group III-V semiconductor compound; and

bonding a face plate to the wafer structure.

2. The method of claim 1, forming the wafer structure further comprising:

growing a third sublayer having a third concentration of the group III-V semiconductor compound.

3. The method of claim 2 wherein the first concentration is less than the second concentration and the second concentration is less than the third concentration.

4. The method of claim 1 wherein the first concentration is less than the second concentration.

5. A method for forming a wafer structure for a photocathode, comprising:

forming an active layer outwardly of a substrate, the active layer comprising a plurality of sublayers, each sublayer having an associated concentration of a group III-V semiconductor compound; and

forming a window layer outwardly of the substrate and the active layer.

6. The method of claim 5, the concentration associated with a specified sublayer based on a placement value for the specified sublayer, the placement value indicative of a number of intervening sublayers between the specified sublayer and the window layer, and wherein the concentration increases as the placement value increases.

7. The method of claim 5, further comprising:

forming a stop layer outwardly of the substrate, the stop layer comprising aluminum gallium arsenide having a concentration of at least about 45% aluminum; and  
wherein forming the active layer comprises forming the active layer outwardly of the stop layer.

8. The method of claim 5, further comprising forming a cap layer outwardly of the window layer, the cap layer comprising gallium arsenide.

9. The method of claim 5, further comprising forming an anti-reflection coating layer outwardly of the window layer, the anti-reflection coating layer comprising silicon nitride.

10. The method of claim 5, forming the active layer comprising:

forming a first sublayer outwardly of the substrate, the first sublayer comprising indium gallium arsenide, the concentration associated with the first sublayer comprising about 15% indium;

forming a second sublayer outwardly of the substrate and the first sublayer, the second sublayer comprising indium gallium arsenide, the concentration associated with the second sublayer comprising about 10% indium; and

forming a third sublayer outwardly of the substrate, the first sublayer and the second sublayer, the third sublayer comprising indium gallium arsenide, the concentration associated with the third sublayer comprising about 5% indium.

11. The method of claim 5, forming the active layer comprising forming each sublayer with a thickness of about 0.5 to about 1.0 microns.

12. The method of claim 5, forming the active layer comprising doping each sublayer with a p-type impurity at a concentration of about  $1 \times 10^{-18}$  to about  $9 \times 10^{-18} \text{ cm}^{-3}$ .

13. A method of making a photocathode, comprising:

providing a substrate;  
forming an active layer outwardly of the substrate, the active layer comprising a plurality of sublayers, each sublayer having an associated concentration of a group III-V semiconductor compound;

forming a window layer outwardly of the substrate and the active layer;

bonding a face plate to the window layer; and  
removing the substrate.

14. The method of claim 13, the concentration associated with a specified sublayer based on a placement value for the specified sublayer, the placement value indicative of a number of intervening sublayers between the specified sublayer and the window layer, and wherein the concentration increases as the placement value increases.

**9**

**15.** The method of claim **13**, further comprising:  
 forming a stop layer outwardly of the substrate; and  
 wherein forming the active layer comprises forming the  
 active layer outwardly of the stop layer;  
 forming a cap layer outwardly of the window layer, the  
 cap layer operable to protect the window layer;  
 removing the cap layer; and  
 forming an anti-reflection coating layer outwardly of the  
 window layer.

**16.** The method of claim **15**, bonding a face plate to the  
 window layer comprising bonding the face plate to the  
 window layer with thermal compression bonding, and fur-  
 ther comprising:

removing the stop layer; and  
 forming an electrode, the electrode coupled to the face  
 plate, the active layer, the window layer, and the  
 anti-reflection coating.

**17. The method of claim 16,**

forming the stop layer comprising forming the stop layer  
 with a thickness of about 1.0 to about 1.5 microns, the  
 stop layer comprising aluminum gallium arsenide hav-  
 ing a concentration of at least about 45% aluminum;  
 forming the window layer comprising forming the win-  
 dow layer with a thickness of about 0.8 to about 1.0  
 microns, the window layer comprising aluminum gal-  
 lium arsenide; and  
 forming the anti-reflection coating layer comprising form-  
 ing first and second antireflection coating layers each

**10**

with a thickness of about 1,000 Å, the first anti-  
 reflection coating layer comprising silicon nitride and  
 the second anti-reflection coating layer comprising  
 silicon dioxide.

**18. The method of claim 13, forming the active layer**  
 comprising:

forming a first sublayer outwardly of the substrate, the  
 first sublayer comprising indium gallium arsenide, the  
 concentration associated with the first sublayer com-  
 prising about 15% indium;

forming a second sublayer outwardly of the substrate and  
 the first sublayer, the second sublayer comprising  
 indium gallium arsenide, the concentration associated  
 with the second sublayer comprising about 10%  
 indium; and

forming a third sublayer outwardly of the substrate, the  
 first sublayer and the second sublayer, the third sub-  
 layer comprising indium gallium arsenide, the concen-  
 tration associated with the third sublayer comprising  
 about 5% indium.

**19. The method of claim 13, forming the active layer**  
 comprising forming each sublayer with a thickness of about  
 0.5 to about 1.0 microns.

**20. The method of claim 13, forming the active layer**  
 comprising doping each sublayer with a p-type impurity at  
 a concentration of about  $1 \times 10^{-18}$  to about  $9 \times 10^{-18} \text{ cm}^{-3}$ .

\* \* \* \* \*